

## UNITED STATES PATENT OFFICE

2,596,978

## 8-HYDROXY-1,2,3,4-TETRAHYDROQUINOLINE AS A SILVER HALIDE DEVELOPER

Robert R. Burtner, Skokie, and Robert T. Dillon,  
Wilmette, Ill., assignors to G. D. Searle & Co.,  
Skokie, Ill., a corporation of Illinois

No Drawing. Application September 17, 1947,  
Serial No. 774,678

9 Claims. (Cl. 95—88)

1

This invention relates to new photographic developer compositions and to solutions thereof, and to the preparation of the same. More particularly, the invention relates to photographic developer compositions containing 8-hydroxy-1,2,3,4-tetrahydroquinoline and homologs thereof for the development of a latent image in a silver halide emulsion.

It is an object of this invention to provide dry powder photographic developer compositions. It is a further object to provide new developing solutions and baths which may be readily prepared and which are stable for extended periods of time. It is still another object of this invention to prepare single powder photographic developers which contain both organic developing agents and alkaline compounds which are suitable for preparing stable aqueous solutions. A further object of this invention is to provide rapid high-energy developing solutions.

We have discovered that photographic developer compositions containing 8-hydroxy-1,2,3,4-tetrahydroquinoline and homologs thereof are extraordinarily stable in neutral and alkaline solutions, and produce extremely rapid photographic developers of high energy. We have further discovered that compositions containing 8-hydroxy-1,2,3,4-tetrahydroquinoline are useful photographic compositions in a variety of solutions, either alone or in combination with other developing agents such as hydroquinone, pyrogallol, catechol, p-aminophenol, p-methylaminophenol, o- and p-phenylenediamine, chlorohydroquinone, bromohydroquinone, and 2,4-diaminophenol. Other 8-hydroxytetrahydroquinolines which are suitable for the preparation of photographic developer compositions include 8-hydroxy-2-methyl-1,2,3,4-tetrahydroquinoline and 8-hydroxy-6-methyl-1,2,3,4-tetrahydroquinoline. The range of tones which can be produced with photographic developer solutions containing 8-hydroxy-1,2,3,4-tetrahydroquinoline runs from brown in the weaker solutions to black in the more concentrated solutions. For this reason the developing solutions which comprise this invention are particularly useful for developing bromide prints. Developing solutions containing 8-hydroxy-1,2,3,4-tetrahydroquinoline exhibit unusual stability; for example, a solution made with sodium sulfite of pH of about 8 is stable for at least one month. Solutions of higher pH are somewhat less stable, as would be expected, but even those made with free sodium hydroxide have remained satisfactory for periods of 1-2 weeks.

Photographic developing compositions containing 8-hydroxy-1,2,3,4-tetrahydroquinoline and homologs thereof are operable in neutral and alkaline solutions. The preferred pH range is about 8.5, although suitable formulations can be made in neutral or very slightly alkaline solu-

2

tions. At higher pH's the 8-hydroxy-1,2,3,4-tetrahydroquinoline is more soluble, and solutions are more readily prepared. Similarly, the speed of development is greater at higher pH values than at neutrality. In our developer compositions, we have found that a variety of alkalies are suitable, such as sodium carbonate, potassium carbonate, sodium hydroxide, trisodium phosphate, borax, sodium sulfite, sodium metaborate and triethanolamine. Inorganic reducing agents which have been found satisfactory for incorporation into our photographic developer solutions include sodium sulfite, sodium bisulfite, potassium thiocyanate, sodium thiocyanate, organic sulfonates, potassium metabisulfite, and potassium ferric oxalate.

We have also discovered that 8-hydroxy-1,2,3,4-tetrahydroquinolines can be readily and efficiently obtained by the catalytic hydrogenation of the corresponding 8-hydroxyquinolines. The reactions can be carried out in any of the solvents known to be suitable for hydrogenation, such as the lower alcohols, the lower saturated hydrocarbons, dioxane, certain non-volatile ethers and other inert solvents. As catalysts we prefer to use Raney nickel because of its ready availability, convenience and efficiency. Other nickel catalysts are also effective, among them being supported nickel catalysts such as nickel on kieselguhr. Noble metal catalysts are suitable also, among them being platinum oxide, palladium black, palladium on charcoal, platinum sponge and the like. The hydrogenation may be carried out over a wide range of temperature and pressure. For example temperatures of 20° to 100° C. and pressures of 20 lb. to 500 lb. are suitable.

Our invention is further disclosed by the following examples, which illustrate typical developing solutions and compositions. Our invention is not to be construed as limited by these examples, which are provided for purposes of illustration only. It will be apparent to those skilled in the photographic arts that a great number of variations in the relative amounts of materials in the formulations may be made without departing from the scope of our invention.

## Example 1

29 grams of 8-hydroxyquinoline in 125 cc. of dioxane are hydrogenated in the presence of Raney nickel at 20-50 lb. pressure at room temperature in 15-20 hours. The hydrogen up-take ceases when it reaches approximately 0.4 mole. Then the catalyst is removed by filtration and the solvent is evaporated under reduced pressure to about  $\frac{1}{3}$  volume. 500 cc. of cold water are added and the precipitated 8-hydroxy-1,2,3,4-tetrahydroquinoline is collected on a filter and dried. After recrystallization from benzene the product melts at 120° C.

In a similar way, 8-hydroxyquinaldine can be reduced to 8-hydroxy-2-methyl-1,2,3,4-tetrahydroquinoline. Other solvents which are suitable include the lower alcohols and hydrocarbons of boiling point 50-150° C.

*Example 2*

A solution of 1.5 g. of 8-hydroxy-1,2,3,4-tetrahydroquinoline in 10 milliliters of ethanol is added to a solution of 25 g. of sodium sulfite, 25 g. of sodium carbonate and 2 to 5 g. of potassium bromide in 800 ml. of water. After mixing, sufficient water is added to bring the volume to 1 liter. The resulting clear solution develops prints of brownish color especially suitable for gold tones.

*Example 3*

A solution of 1 g. of 8-hydroxy-1,2,3,4-tetrahydroquinoline in 10 ml. of ethanol is added to a solution of 25 g. of sodium sulfite and 2 to 5 g. of potassium bromide in 500 ml. of N/10 sodium hydroxide solution. After mixing, sufficient water is added to bring the volume to 1 liter. The resulting clear solution forms brown-black prints.

*Example 4*

A solution of 0.5 g. of 8-hydroxy-1,2,3,4-tetrahydroquinoline and 0.5 g. of p-methylaminophenol in 10 ml. of ethanol is added to a solution of 25 g. of sodium sulfite, 25 g. of sodium carbonate and 3 g. of potassium bromide in 800 ml. of water. The resulting solution is brought to 1 liter with additional water. The clear solution is a high energy developer which produces grey-black prints.

*Example 5*

A solution of 0.5 g. of 8-hydroxy-1,2,3,4-tetrahydroquinoline and 0.5 g. of hydroquinone in 10 ml. of ethanol is added to a solution of 25 g. of sodium sulfite and 2 to 5 g. of potassium bromide in 500 ml. of N/10 sodium hydroxide solution. After mixing, sufficient water is added to bring the volume to 1 liter. This developer gives black prints of good contrast and clear whites.

*Example 6*

A 2.5% aqueous solution of sodium sulfite is warmed slightly and saturated with 8-hydroxy-1,2,3,4-tetrahydroquinoline (approximately 0.5 g. per liter). The resulting clear solution is filtered and provides a neutral developing solution of great stability.

*Example 7*

2 g. of 8-hydroxy-1,2,3,4-tetrahydroquinoline in 100 ml. of hot water are added to 800 ml. of water containing 25 g. of sodium sulfite, 5 g. of hydroquinone and 2 g. of borax. Sufficient water is added to bring the volume of the resulting solution to 1 liter. The resulting high energy developer is stable for 2-3 weeks.

*Example 8*

A dry powder mixture is prepared by thoroughly mixing the following materials:

|                                       | Grams |
|---------------------------------------|-------|
| 8-hydroxy-1,2,3,4-tetrahydroquinoline | 6     |
| Hydroquinone                          | 24    |
| Sodium carbonate monohydrate          | 216   |
| Potassium metabisulfite               | 111   |
| Potassium bromide                     | 12    |
| Sodium sulfite                        | 90    |

This mixture can be dissolved with slight warming in 4 liters of water to make a stable stock developer solution which is unchanged for at least a week. The dry powder may be stored for 5 several months without change.

*Example 9*

To a solution of 1 g. of 8-hydroxy-1,2,3,4-tetrahydroquinoline in 200 ml. of N/10 sodium hydroxide solution are added 25 g. of sodium sulfite and 5 g. of potassium bromide in 500 ml. of water. After thorough mixing the resulting clear solution is diluted to 1 liter with water. It develops light-hued brown prints.

We claim:

1. A photographic developing composition for the development of a latent image in a silver halide emulsion comprising an 8-hydroxy-1,2,3,4-tetrahydroquinoline and a soluble inorganic reducing agent containing tetravalent sulfur.
2. A photographic developing composition comprising an 8-hydroxy-1,2,3,4-tetrahydroquinoline and sodium sulfite.
3. A photographic developing composition for the development of a latent image in a silver halide emulsion comprising an 8-hydroxy-1,2,3,4-tetrahydroquinoline, a hydroquinone and a soluble inorganic sulfite.
4. A photographic developing composition comprising an 8-hydroxy-1,2,3,4-tetrahydroquinoline, a hydroquinone and sodium sulfite.
5. A photographic developing solution comprising an aqueous solution of an 8-hydroxy-1,2,3,4-tetrahydroquinoline and sodium sulfite.
6. A photographic developing solution comprising an aqueous solution of an 8-hydroxy-1,2,3,4-tetrahydroquinoline, a hydroquinone and sodium sulfite.
7. In a process of developing a latent image of an exposed silver halide emulsion, the step which comprises treating said emulsion with an aqueous solution containing an 8-hydroxy-1,2,3,4-tetrahydroquinoline and a soluble inorganic reducing agent containing tetravalent sulfur.
8. In a process of developing a latent image of an exposed silver halide emulsion, the step which comprises treating said emulsion with an aqueous solution containing an 8-hydroxy-1,2,3,4-tetrahydroquinoline, a hydroquinone and a soluble inorganic sulfite.
9. In a process of developing a latent image of an exposed silver halide emulsion, the step which comprises treating said emulsion with an aqueous solution containing an 8-hydroxy-1,2,3,4-tetrahydroquinoline and sodium sulfite.

ROBERT R. BURTNER  
ROBERT T. DILLON

REFERENCES CITED

The following references are of record in the file of this patent:

UNITED STATES PATENTS

| Number    | Name            | Date          |
|-----------|-----------------|---------------|
| 2,108,243 | Wendt           | Feb. 15, 1938 |
| 2,163,820 | Wilmanns et al. | June 27, 1939 |
| 2,194,399 | Lange           | Mar. 19, 1940 |
| 2,251,922 | Dickey et al.   | Aug. 12, 1941 |
| 2,328,034 | Sease et al.    | Aug. 31, 1943 |